

## UNITED STATES PATENT OFFICE.

ADOLPHE H. NEY, OF NEW YORK, N. Y.

## FLOTATION OF ORES.

No Drawing.

Application filed December 27, 1926. Serial No. 157,407.

This invention relates to a new and improved process for the concentration of ores by the method known as "fotation" and particularly to the use and employment, in 5 said ore concentration process, of chemicals and substances and transformation products thereof, hitherto unknown as being of advantage and utility as agents or assisting and auxiliary substances in said ore concentration process as customarily practiced.

The process of concentrating ore commonly designated "fotation" consists in producing by suitable means upon the surface of an aqueous suspension of a finely 15 comminuted ore body, a froth. Under suitable conditions, this froth carries to the surface of the liquid a "concentrate" containing a higher percentage of the metallic or other valuable constituents of the ore 20 treated than it originally contained. This concentrate is continuously or intermittently removed and further treated to recover and purify its valuable constituents.

A variety of substances has been hitherto 25 proposed and employed as agents or assisting and auxiliary media for producing the "concentrating" effect and many of these substances known as "fotation agents" are indeed effective in a greater or lesser degree 30 in that their addition to or presence in the operation of flotation produces or effects the formation of a "concentrate" having a higher percentage of the valuable constituents of the ore treated than the latter originally 35 contained. The relative value of such flotation agents also depends on the amount necessary to be effective and on the time required to produce such effect, and their price.

40 I have discovered that a new series of compounds hitherto not employed for this purpose are very efficient flotation agents surpassing in their effectiveness any proposed and known substances in producing a high concentrate. These substances are the 45 products of reaction of disulfurdichloride in excess upon aromatic amino compounds having at least one ortho-position to the amino group free or unsubstituted. These 50 reaction products are described for instance in British patent specifications No. 17,417 of 1914 and 18,292 of 1914, and are by suitable treatment with water and alkali transformed into o-amidothiophenol like bodies.

To illustrate the use of these substances 55 the following example is given.

## Example.

1000 grams of a copper bearing ore, containing 1.2% Cu are ground to fineness of 60 #60 mesh with some water, 5 grammes slaked lime and 0.125 grammes of the product of reaction between disulfurdichloride and orthotoluidine being added. The mixture was placed into a flotation test machine, water added and aeration started. Five drops of pine oil were added as needed during the operation. The froth was removed as formed and aeration continued for fifteen minutes. The froth when dried weighed 60 grammes and contained 10.2 grammes copper. An extraction of 85% of the copper present in the ore was thus effected and a 17% concentrate obtained.

Similar results can be obtained on a large 75 scale by appropriate methods of operation and suitable apparatus.

It is understood that my invention is not limited to the proportion of materials used in the example given nor to the nature of 80 the subsidiary agents. Neither do I wish to be restricted to the use of any particular method or modus of working or operation, or to any particular type of apparatus or machinery, all these things being capable of 85 variation and modification according to the nature of the ore treated and the result desired.

Inasmuch as the aforementioned products of reaction of disulfurdichloride and aromatic amines react with water under formation of new bodies and liberation of hydrochloric acid and, inasmuch as the latter new bodies are under the influence of alkalies in turn transformed into o-amido thiophenol like substances, all of which produce in the flotation operation the same or a similar effect, namely the formation of a high grade concentrate, I may employ the product of "hydrolysis" upon the reaction 90 product of disulfurdichloride and an aromatic amine, or the o-amido thiophenol-like substance obtained by treating the product of "hydrolysis" with alkalies, in any preferred manner. For instance, I may substitute, in the example given, the product of reaction of disulfurdichloride and orthotoluidine by an equivalent or similar quan-

5 tity of the transformation product obtained from said reaction product by dissolving the latter in water and separating from the solution the pinkish white product of hydrolysis which precipitates from such a solution in course of a few hours; or again I may use in place of the product of reaction of disulfurdichloride and ortho-toluidine, a similar amount of the o-amidothiophenol-like body which I obtain by dissolving the hydrolyzed reaction product in an alkali, and isolating from this solution the o-amidothiophenol-like body in any desired manner, as for instance by precipitating it by means 10 of zinc-chloride and decomposing the zinc-salt of the o-amidothiophenol with hydrogen sulphide.

Having thus described the nature of my said invention and in what manner it may 15 be applied, I declare that what I claim is:

20 1. The method of concentrating ores by

froth flotation which comprises subjecting the mineral in form of an alkaline pulp to a froth flotation operation in the presence of the products of reaction of an excess of disulfurdichloride upon aromatic amino compounds having at least one orthoposition to the amino group free or unsubstituted. 25

2. The method of concentrating ores by froth flotation which comprises subjecting the mineral in the form of a pulp rendered alkaline with lime to a froth flotation operation in the presence of the products of reaction of an excess of disulfurdichloride upon aromatic amino compounds having at least one orthoposition to the amino group free or unsubstituted. 30

Signed at New York city, in the county of Kings and State of New York, this twentieth day of December, A. D. 1926.

ADOLPHE H. NEY.